

United States Patent [19]  
Takahashi et al.

[11] 3,865,645  
[45] Feb. 11, 1975

[54] COLD-ROLLED STEEL SHEET FOR  
PRESS-FORMING

[75] Inventors: Nobuyuki Takahashi; Kenitiro  
Suemune; Shuji Nagata; Tatumi  
Tomozoe, all of Kitakyushu, Japan

[73] Assignee: Nippon Steel Corp., Tokyo, Japan

[22] Filed: Dec. 27, 1972

[21] Appl. No.: 319,017

[30] Foreign Application Priority Data

Dec. 27, 1971 Japan ..... 46-10537

[52] U.S. Cl. ..... 148/142, 75/124, 148/2,  
148/12.3, 148/36

[51] Int. Cl. ..... C22c 41/02, C21d 9/48

[58] Field of Search ..... 75/123 R, 123 B; 148/36,  
148/2, 12.3, 134, 143, 142

[56] References Cited

UNITED STATES PATENTS

2,109,271 2/1938 Krause ..... 75/123  
2,125,128 7/1928 Robinson ..... 148/142

|           |         |                |         |
|-----------|---------|----------------|---------|
| 2,319,655 | 5/1943  | Saylov .....   | 75/123  |
| 2,986,403 | 5/1961  | Leslie .....   | 148/12  |
| 3,117,897 | 1/1964  | Williams ..... | 148/142 |
| 3,239,389 | 3/1966  | Yoshida .....  | 75/123  |
| 3,323,953 | 6/1967  | Lesney .....   | 148/39  |
| 3,357,822 | 12/1967 | Miyoshi .....  | 148/142 |

OTHER PUBLICATIONS

"Making Shaping and Treating of Steel," by U.S.  
Steel, 8th Edition, published 1964, pages, 552-554.

Primary Examiner—C. Lovell  
Attorney, Agent, or Firm—Wenderoth, Lind & Ponack

[57] ABSTRACT

A cold-rolled steel sheet having an excellent  
press-formability, consisting of less than 0.08 wt. per-  
cent carbon, 0.05 to 0.4 wt. percent manganese, 0.015  
to 0.10 wt. percent silicon, 0.01 to 0.10 wt. percent  
acid-soluble aluminum, 0.003 to 0.015 wt. percent ni-  
trogen, the balance being iron and unavoidable impu-  
rities, said cold-rolled steel sheet being manufactured  
through a process step of a continuous annealing with  
or without an overaging treatment.

5 Claims, 1 Drawing Figure

PATENTED FEB 11 1975

3,865,645



## COLD-ROLLED STEEL SHEET FOR PRESS-FORMING

The present invention relates to a cold-rolled steel sheet for press-forming, manufactured by a continuous annealing.

In general, cold-rolled steel sheets are used as such parts of automobiles as cold-formed by a drawing working, for instance, rear fender, front fender and door inner, for which an excellent drawing workability is required.

As for cold-rolled steel sheets having such an excellent drawing workability there are used at present an aluminum-killed low carbon steel containing 0.03 to 0.07 wt. percent carbon and 0.02 to 0.08 wt. percent acid-soluble aluminum and further a cold-rolled titanium-added extremely low carbon steel sheet, in which the drawing workability is not influenced by a rate of heating of an annealing and is superior to the aluminum-killed low carbon steel sheet, due to the fixation of carbon and nitrogen by titanium. However, this aluminum-killed low carbon steel sheet is almost annealed in the state of a tight coil or of an open coil by using a box annealing furnace. But, such a box annealing has following disadvantages: a long time is required for annealing, the productivity is low and a uniform heating of the whole coil or of the interior of the furnace is not obtainable for a constructional reason, whereby a uniform material quality over the whole length of coil can not be achieved. Particularly, in the case of an annealing in the state of a tight coil the contact between the surface of a steel sheet and an atmosphere gas within the furnace is bad and moreover there occur easily various kinds of hindrances in regard to the surface properties due to lack of the uniformity. Further, a titanium-added extremely low carbon steel sheet has a disadvantage that its production cost becomes higher than that of an aluminum-killed low carbon steel, because the former contains about 0.1 wt. percent titanium.

These problems caused in subjecting an aluminum-killed cold-rolled steel sheet to a box annealing are solved by a continuous annealing to be conducted in a continuous annealing furnace. In general, a continuous annealing has following advantages: the productivity is high for reason of construction; a uniformity of material qualities through one coil and that between coils are obtained; and a uniform contact between the surface of a steel sheet and atmosphere gas within the furnace is secured. However, on the other hand, the continuous annealing can not be freed from disadvantages: that is, on account of a rapid heating and a short soaking time crystal grains are refined in general, and on account of a high rate of cooling subsequent to the annealing carbon contained in the steel can not sufficiently precipitate as carbide so that the continuously annealed steel is high in yield stress and tensile strength, but low in breaking elongation and n-value and great in aging property as compared with a box-annealed steel material. Therefore, the former is inferior to the latter in the press-formability. Therefore, the continuous annealing treatment is usually not applied to the production of a cold-rolled steel sheet for press-forming, but mainly for the production of steel sheet to be used as material for producing tin plate.

Reasons, why a cold-rolled steel sheet subjected to a continuous annealing treatment has an unfavorable

press-formability, are found in the following situations: on account of rapid heating and short annealing time crystal grains are difficult to grow, but are easy to refine; on account of a quenching after the annealing, the

5 amount of solid solution of carbon is large, so that there is caused a hardening aging, which makes the steel material hard, and finally on account of rapid heating, the development of a recrystalline collective texture, which is essentially desirable for the drawability, is checked.

10 However, the greatest problem, with which the production of a cold-rolled steel sheet for drawing of such qualities as of the SPCD class prescribed in the Japanese Industrial Standard (JIS) is confronted, is hardening aging due to quenching.

15 As a method for preventing a steel material from becoming hard on account of a hardening aging, there has been adopted method, in which a steel sheet coil

20 quenched after the continuous annealing is successively subjected to a heat treatment (overaging treatment) at a temperature of 300° to 500°C. in a continuous annealing furnace or a box annealing furnace. However, in case the continuous annealing is followed by the overaging treatment in a box annealing furnace, the productivity of the annealing is reduced and the original aim of carrying out the continuous annealing must be lost.

25 However, even when carrying out the overaging treatment continuously in a continuous annealing furnace a sufficient softening of the steel material is still 30 difficult to obtain, if the overaging treatment of an economic or practical scale (for instance, the overaging treatment for less than 10 minutes) is conducted.

As a result of numerous investigations made by the inventors of the present invention on chemical compositions of steel sheets for promoting the overaging phenomenon it was confirmed that, when a usual aluminum-killed low carbon steel contains an adequate amount of silicon, the overaging rate is quickened, 35 whereby the steel material is made soft, even with an overaging treatment of a short time, and a cold-rolled steel sheet for press-forming can be produced.

It has been further confirmed by the same inventors of the present invention that by subjecting the above- 40 mentioned aluminum-killed low carbon steel sheet to vacuum degassing treatment to reduce the C content to 0.001 to 0.009 percent there can be obtained a cold-rolled steel sheet, in which the drawing workability and stretching workability are of the same degree as a 45 titanium-added extremely low carbon steel sheet and the drawing workability is not influenced by the heating rate of the annealing.

50 Therefore, the object of the present invention is to produce a cold-rolled steel sheet having an excellent press-formability when subjected to a continuous annealing.

Another object of the present invention is to provide a cold-rolled steel sheet having an excellent press-formability by the application of an overaging treatment of 55 a continuous annealing system.

A still another object of the present invention is to provide a cold-rolled steel having always an excellent drawing workability without being influenced by a rate of cooling subsequent to a hot-rolling and a cooling 60 temperature by subjecting the said steel to a vacuum degassing treatment to reduce the C content to 0.001 to 0.009 percent.

Another object of the present invention shall be made clear by the following explanation with reference to an attached drawing.

The attached drawing shows influences of silicon contents on changes in properties of steel materials, when subjecting aluminum-killed low carbon steel sheets having different silicon contents to an overaging treatment of the continuous annealing.

The steel sheet of the present invention is a cold-rolled steel sheet having an excellent press-formability, said steel consisting of less than 0.08 wt. percent carbon, 0.05 to 0.4 wt. percent manganese, 0.015 to 0.10 wt. percent silicon, 0.01 to 0.1 wt. percent acid-soluble aluminum, 0.003 to 0.015 wt. percent nitrogen and the rest being iron and unavoidable impurities.

At first, the components of the steel sheet of the present invention shall be explained.

The carbon content of the steel sheet of the present invention is the same as that of a cold-rolled low carbon steel of the SPCC class (cold-rolled steel sheet in general) or the SPCD class (cold-rolled steel sheet for drawing) prescribed by G 3141 of the JIS. It is not particularly necessary to reduce the carbon content for mitigating the hardening aging. However, in case properties of the same degree as of a titanium-added extremely low carbon steel sheet is required for the steel sheet of the present invention its carbon content is reduced to 0.001 to 0.009 wt. percent by subjecting the steel to a vacuum degassing treatment.

Manganese Mangan must be contained for the purpose of preventing a brittle rupture caused by sulfur at the time of hot-rolling. In view of the fact that an aluminum-killed steel prepared by melting in a converter contains usually sulfur in an amount of more than 0.005 percent, the manganese content must be more than 0.05 percent in order to fix the above-mentioned amount of sulfur. But, since an excessive amount of manganese brings about a deterioration of the workability of the steel, the upper limit thereof is made 0.4 percent.

Silicon is contained usually in an amount of less than 0.01 percent in a cold-rolled steel sheet refined in a steel making furnace prescribed in G 3141 of the JIS. However, in the steel of the present invention the silicon content is necessary to be in an amount of more than 0.015 percent, preferably more than 0.02 percent, in order to obtain properties of a steel sheet for press-forming (of SPCD class of JIS) by a continuous annealing comprising an overaging treatment, without being influenced by conditions of production steps (for instance, hot-rolling condition) prior to the cold-rolling.

However, when the silicon content exceeds 0.1 percent, the strength of the steel sheet is increased to a degree more than required, whereby the workability is deteriorated. Therefore, the upper limit thereof is made 0.1 percent.

In connection with the silicon content, as above-mentioned, it is to note that there is a mutual relationship between the silicon content and the carbon content. It has been confirmed by the inventors of the present invention that in the case of the steel of the present invention containing silicon in a range of 0.015 to 0.1 percent it is preferable to reduce the carbon content to a level of less than 0.009 percent by subjecting the steel to a vacuum degassing treatment in order to liberate the  $\bar{r}$ -value, that is, an average value of the plastic strain ratio, which serves as an index of the drawability of the

steel, from the dependency of the heating rate of annealing. However, if the silicon content is below the range as above-mentioned, the  $\bar{r}$ -value can not be liberated from the dependency on the heating rate of annealing, even if the carbon content is in the range of from 0.001 to 0.009 percent, as specified by the present invention.

Further, also a phenomenon that, when the silicon content is more than 0.015 percent, the drawability is 10 liberated from being influenced by a coiling temperature of annealing indicates that there is a relationship between the carbon content and silicon content.

Further, in order to achieve the object of the present invention it is necessary to contain an acid-soluble aluminum in an amount of more than 0.01 percent. However, the lower limit of the acid-soluble aluminum desirable to prevent the occurrence of stretcher strain caused by oxides contained in the steel is defined to be 0.02 percent. On the other hand, if the acid-soluble aluminum exceeds 0.1 percent, the workability of the steel 20 is deteriorated. Therefore, the upper limit thereof is made 0.1 percent.

In order to mitigate the hardening due to a hardening aging of cold-rolled steel sheet subjected to a continuous annealing treatment, that is, to quicken the overaging rate, the co-presence of three components, that is, silicon, aluminum and nitrogen, is more effective than a sole presence of silicon. For this purpose nitrogen is necessary to be contained in an amount of more than 25 0.003 percent. However, if exceeds 0.015 percent, the workability is deteriorated. Therefore, the upper limit thereof is made 0.015 percent.

As is evident from the foregoing, the prerequisite conditions for achieving the object of the present invention 30 is the limitation of four basic chemical components: carbon, silicon, aluminum and nitrogen, for reasons as above-mentioned.

The steel sheet of the present invention is manufactured by the steps of refining a molten steel in a steel-making furnace such as converter, open hearth furnace, electric furnace, an ingot-making, a slab-making by blooming or a continuous casting and subsequent hot-rolling. The finishing temperature of the hot-rolling is preferable to be higher than 800°C. A coiling temperature is not limited. That is, in the case of an aluminum-killed low carbon steel the drawing workability of the steel can not be obtained, unless the steel is heated to a grain coarsening point as a finishing temperature of hot-rolling and rapidly cooled after the hot-rolling, for 40 reason that the drawability will be deteriorated on account of AlN precipitating at grain boundaries or coiled at a temperature near the  $A_1$  transformation point.

On the contrary, in the present invention neither the 55 finishing temperature of the hot-rolling nor coiling temperature has influence on the effects of components of the steel of the present invention for promoting the overaging. The thus obtained hot-rolled coil is then subjected to a cold-rolling after it was scaled. The reduction percentage of the cold-rolling must be more than 30 percent, preferably 60 to 85 percent, from the view point of the drawing workability.

The cold-rolled coil is then annealed in a continuous annealing furnace with an adequate heating system.

60 The annealing temperature is higher than 680°C., but lower than 900°C., and the time required for the soaking is less than 10 minutes. The annealed coil is then

subjected to an overaging treatment in a apparatus for overaging treatment under conditions of a temperature of 300° to 500°C, and a time of less than 10 minutes, preferably 2 to 5 minutes. Further, in the case of the steel of the present invention the rate of cooling from the annealing temperature to the overaging treatment temperature exerts no influence on the effect of the overaging treatment.

After the overaging treatment the steel sheet is then subjected to an adequate method such as refining-rolling or passing-through a leveler to regulate its shape and eliminate yield point elongation.

In the following the present invention shall be explained by example.

#### EXAMPLE 1

Table 1 shows chemical components of steel materials of various kinds for explaining examples of the present invention.

These steel materials were cold-rolled to the sheet gauge of 0.8mm. through usual process steps of producing cold-rolled steel sheets under hot-rolling and cold-rolling conditions as shown in Table 2. Thereafter, the steel materials were annealed at 700°C. for 3 minutes in a continuous annealing furnace after up to 20 700°C. in a minute. After the annealing the steel materials were cooled down to 370°C. by any of cooling rates shown in Table 3 and then were subjected to an overaging treatment at 430°C. for 5 minutes. Further, each of the steel materials was subjected to a refining rolling with a reduction percentage of 1.5 percent. Mechanical properties of the cold-rolled steel sheets obtained through the above-mentioned process steps are shown in Table 4.

tents were subjected to a continuous annealing. Then, a part of them were subjected to the overaging treatment, while another part of them were not. The mechanical properties of the steels were investigated in comparison of both cases, and the results of the investigations are shown in Figure.

The composition of steel samples subjected to the investigations and the treatment conditions are as follows:

- 10 1. Composition
 

|                               |
|-------------------------------|
| C : 0.04 – 0.07 percent       |
| Mn : 0.18 – 0.30 percent      |
| Sol. Al : 0.04 – 0.06 percent |
| N : 0.0045 – 0.0060 percent   |
- 15 2. Hot-rolling conditions
 

|                                     |
|-------------------------------------|
| Finishing temperature : 890 ± 10°C. |
| Coiling temperature: 630 ± 10°C.    |
3. Cold-rolling condition
 

|                                   |
|-----------------------------------|
| Reduction percentage : 73 percent |
|-----------------------------------|
4. Continuous annealing conditions
 

|                                             |
|---------------------------------------------|
| Soaking condition : 700°C. × 90 sec.        |
| Rate of heating-up : 60 sec. till to 700°C. |
| Rate of cooling : Average 22°C./sec.        |
| Overaging treatment : 350°C. × 5 min.       |
5. Refining rolling 5.
 

|                                    |
|------------------------------------|
| Reduction percentage : 1.5 percent |
|------------------------------------|

As is seen from the attached drawing, if steel sheets contain silicon in an amount of more than 0.01 percent, a remarkable softening of the steel materials under the same overaging treatment conditions is obtained, whereby a press-formability is so strikingly improved that the material qualities obtained thereby are closely allied to those of SPCD class of the JIS which are subjected to a box annealing.

Table 1

| Coil No.                                              | C | Mn   | Si   | P     | S    | Chemical composition |       |              |
|-------------------------------------------------------|---|------|------|-------|------|----------------------|-------|--------------|
|                                                       |   |      |      |       |      | Sol. Al              | N     | O            |
| Steel sheet within the range of the present invention | A | 0.05 | 0.15 | 0.032 | 0.02 | 0.01                 | 0.053 | 0.0038 0.005 |
|                                                       | B | 0.03 | 0.33 | 0.020 | 0.02 | 0.02                 | 0.040 | 0.0048 0.008 |
|                                                       | C | 0.06 | 0.20 | 0.047 | 0.03 | 0.02                 | 0.032 | 0.0068 0.007 |
|                                                       | D | 0.05 | 0.23 | 0.017 | 0.01 | 0.01                 | 0.080 | 0.0059 0.004 |
|                                                       | E | 0.02 | 0.29 | 0.080 | 0.04 | 0.02                 | 0.057 | 0.0045 0.006 |
|                                                       | F | 0.06 | 0.19 | 0.023 | 0.02 | 0.01                 | 0.045 | 0.0056 0.010 |
| Steel sheet out of the range of the present invention | G | 0.05 | 0.32 | 0.009 | 0.01 | 0.01                 | 0.053 | 0.0049 0.005 |
|                                                       | H | 0.04 | 0.28 | 0.035 | 0.02 | 0.02                 | 0.006 | 0.0029 0.018 |
|                                                       | I | 0.05 | 0.31 | 0.010 | 0.02 | 0.02                 | 0.002 | 0.0019 0.032 |
|                                                       | J | 0.07 | 0.32 | 0.024 | 0.01 | 0.02                 | 0.045 | 0.0024 0.011 |
|                                                       | K | 0.04 | 0.30 | 0.010 | 0.02 | 0.02                 | 0.054 | 0.0058 0.006 |

Cold-rolled steel sheets containing acid-soluble aluminum, nitrogen and silicon in amounts within the ranges specified by the present invention are in general softer than those containing these components in amounts out of the said respective ranges and are excellent in all of the breaking elongation, *n*-value and *r*-value. Therefore, it is clear that the steel sheets of the present invention have very good press-formability. At the same time it is to note that the mechanical properties of the steels of the present invention are little influenced by the cooling temperature of hot-rolling and the range of cooling after the annealing.

#### Example 2

With an aim of investigating the influence of silicon on the effect of the overaging treatment aluminum-killed low carbon steels having different silicon con-

Table 2

| Coil No. | Rolling record              |                     |                               |
|----------|-----------------------------|---------------------|-------------------------------|
|          | Hot-rolling conditions (°C) |                     | Cold-reduction percentage (%) |
|          | Finishing temperature       | Coiling temperature |                               |
| A        | 890                         | 560                 | 73                            |
| B        | 880                         | 560                 | 73                            |
| C        | 850                         | 560                 | 73                            |
| D        | 870                         | 680                 | 73                            |
| E        | 900                         | 680                 | 73                            |
| F        | 890                         | 680                 | 73                            |
| G        | 865                         | 680                 | 73                            |
| H        | 890                         | 560                 | 73                            |
| I        | 880                         | 680                 | 73                            |
| J        | 890                         | 680                 | 73                            |
| K        | 880                         | 560                 | 73                            |

7  
Table 3

| Cooling condition down to 430°C after the annealing at 700°C |                                |
|--------------------------------------------------------------|--------------------------------|
| Cooling system                                               | Average cooling rate (°C/sec.) |
| I                                                            | 5.4 (Time required: 50 sec.)   |
| II                                                           | 22.5 (Time required: 12 sec.)  |
| III                                                          | 54.0 (Time required: 5 sec.)   |

8  
Table 6

| 5 | Coil No. | Hot-rolling conditions (°C) |                     | Cold-reduction percentage (%) |
|---|----------|-----------------------------|---------------------|-------------------------------|
|   |          | Finishing temperature       | Coiling temperature |                               |
|   | A        | 890                         | 560                 | 70                            |
|   | B        | 880                         | 530                 | 70                            |

Table 4

| Mechanical properties                                             |          |                |                                   |                                        |                |         |         |
|-------------------------------------------------------------------|----------|----------------|-----------------------------------|----------------------------------------|----------------|---------|---------|
|                                                                   | Coil No. | Cooling system | Yield point (kg/mm <sup>2</sup> ) | Tensile strength (kg/mm <sup>2</sup> ) | Elongation (%) | n-value | r-value |
| Cold-rolled steel sheet within the range of the present invention | A        | I              | 22.5                              | 33.2                                   | 44.0           | 0.236   | 1.40    |
|                                                                   | B        | II             | 21.3                              | 32.5                                   | 44.3           | 0.240   | 1.42    |
|                                                                   | C        | III            | 22.0                              | 33.2                                   | 43.8           | 0.236   | 1.45    |
|                                                                   | D        | I              | 20.8                              | 32.0                                   | 44.8           | 0.241   | 1.46    |
|                                                                   | E        | II             | 23.0                              | 34.0                                   | 44.0           | 0.237   | 1.47    |
|                                                                   | F        | III            | 19.5                              | 31.2                                   | 45.7           | 0.240   | 1.51    |
| Cold-rolled steel sheet out of the range of the present invention | G        | III            | 23.7                              | 35.3                                   | 41.2           | 0.229   | 1.41    |
|                                                                   | H        | III            | 23.4                              | 34.8                                   | 42.0           | 0.230   | 1.23    |
|                                                                   | I        | III            | 27.3                              | 36.5                                   | 40.1           | 0.225   | 1.08    |
|                                                                   | J        | III            | 24.0                              | 36.0                                   | 42.2           | 0.228   | 1.25    |
|                                                                   | K        | III            | 27.9                              | 37.2                                   | 40.5           | 0.223   | 1.18    |

## Example 3

Table 5 shows steel samples prepared by subjecting the steels having chemical compositions shown in Examples 1 and 2 to a vacuum degassing treatment to re-

|   |     |     |    |
|---|-----|-----|----|
| C | 890 | 620 | 74 |
| D | 870 | 570 | 76 |
| E | 850 | 570 | 70 |
| F | 840 | 390 | 70 |
| G | 900 | 550 | 76 |

Table 7

| Mechanical properties of annealed steel materials |                                                 |                                        |                       |                         |         |         |
|---------------------------------------------------|-------------------------------------------------|----------------------------------------|-----------------------|-------------------------|---------|---------|
| Sample No.                                        | Yield <sup>*4</sup> point (kg/mm <sup>2</sup> ) | Tensile strength (kg/mm <sup>2</sup> ) | Mechanical properties | Breaking elongation (%) | n-value | r-value |
| *1                                                | A                                               | 14.3                                   | 32.6                  | 49                      | 0.259   | 1.94    |
|                                                   | B                                               | 15.0                                   | 32.0                  | 49                      | 0.250   | 1.95    |
|                                                   | C                                               | 15.1                                   | 32.0                  | 49                      | 0.255   | 1.80    |
|                                                   | D                                               | 15.3                                   | 32.5                  | 47                      | 0.254   | 2.00    |
| *2                                                | E                                               | 19.3                                   | 33.5                  | 44                      | 0.238   | 1.53    |
|                                                   | F                                               | 18.2                                   | 35.6                  | 43                      | 0.220   | 1.15    |
| *3                                                | G                                               | 12.8                                   | 31.8                  | 53                      | 0.291   | 2.40    |

\*1: Steel within the range of the present invention

\*2: Steel out of the range of the present invention

\*3: Ti-added extremely low carbon steel out of the range of the present invention

\*4: 0.2% proof stress

Annealing system: Continuous annealing system 870°C×4min.

duce the carbon content to a range of from 0.001 to 0.009 percent.

These steels were hot-rolled and then cold-rolled under usual hot-rolling and cold-rolling conditions as shown in Table 6 to obtain the gauge of 0.8 mm. thereby and thereafter were subjected to continuous annealing at 870°C. for 4 minutes. The thus annealed steel sheets were then subjected to refining rolling with a reduction percentage of 1.0 percent. The mechanical properties of the steel sheets thus produced through the above-mentioned process steps are as shown in Table 7.

Table 5

| Sample No.                                                                      | C | Mn    | Si   | P     | Sol. Al | N     | O      | S     |
|---------------------------------------------------------------------------------|---|-------|------|-------|---------|-------|--------|-------|
| Al-killed, extremely low carbon steel within the range of the present invention | A | 0.007 | 0.15 | 0.032 | 0.02    | 0.043 | 0.0076 | 0.005 |
|                                                                                 | B | 0.005 | 0.33 | 0.020 | 0.02    | 0.086 | 0.0103 | 0.008 |
|                                                                                 | C | 0.009 | 0.30 | 0.065 | 0.02    | 0.097 | 0.0138 | 0.006 |
|                                                                                 | D | 0.004 | 0.10 | 0.145 | 0.01    | 0.027 | 0.0045 | 0.012 |
| Al-killed steel out of the range of the present invention                       | E | 0.013 | 0.28 | 0.030 | 0.02    | 0.043 | 0.0082 | 0.003 |
|                                                                                 | F | 0.008 | 0.23 | 0.010 | 0.03    | 0.03  | 0.0056 | 0.005 |
| Ti-added extremely low carbon steel out of the range of the present invention   | G | 0.008 | 0.15 | 0.01  | 0.01    | 0.105 | 0.0045 | 0.03  |

As is evident from the foregoing, particularly in reference to Examples 1 and 2, the fundamental idea of the present invention, which has for its purpose the provision of a steel sheet having an excellent press-formability by a continuous annealing method, is based on the discoveries that an excellent press-formability can be rendered to the steel sheet subjected to a continuous annealing by specifying main components of the steel, particularly adding silicon in an amount as is specified by the present invention, but the press-formability of steel can be more remarkably improved by subjecting said steel to an overaging treatment, that is, a kind of

an artificial aging which is aimed at the softening of steel material.

Thus, the present invention has succeeded in economically overcoming the greatest problem, the steel material becoming hard due to a hardening aging, encountered in producing a cold-rolled low carbon steel sheet by a continuous annealing according to any conventional methods. The reason, why the overaging rate of the steel sheet of the present invention is quick, seems to lie in the fact that silicon contained in the steel will promote the precipitation of carbide. This is also assumed to be connected with the fact that the  $\bar{r}$ -value of the steel of the present invention acquired after the continuous annealing is little influenced by a cooling temperature of the hot-rolling, because AlN precipitated during the hot-rolling will not take the simple form of AlN, but a compound precipitate of Al-N-C, consequently there would exist no great difference in size of the precipitate and distribution form thereof.

Further, Example 3 teaches that even without subjecting the steel of the present invention to the overaging treatment at the end of the continuous annealing treatment the press-formability may be improved, when the carbon content is reduced to a range of from 0.001 to 0.009 percent to soften the steel by subjecting the molten steel to a vacuum degassing treatment.

In this case it is further to note that the  $\bar{r}$ -value may be also liberated from its dependency on a heating rate of annealing. In general, in the case of a steel containing carbon in an amount of more than 0.01 percent, the dependency of the  $\bar{r}$ -value on the heating rate of annealing varies depending upon the carbon content of the steel, as is special for an aluminum-killed cold-rolled steel sheet. Therefore, by reducing the carbon content of the steel of the present invention to less than 0.09 percent by subjecting the same to a vacuum degassing treatment, as above-mentioned, said dependency of the  $\bar{r}$ -value disappears. This indicates that the recrystallization structure of the aluminum-killed cold-rolled steel sheet undergoes a change from a certain line of carbon content, while making the carbon content of 0.01 percent a boundary line, from which it is understood that the recrystallization structure of the aluminum-killed cold-rolled steel sheet having a carbon content of less than 0.01 percent is suited to an annealing process, in which rapid heating is to be conducted.

What is claimed is:

1. A process for preparing a cold-rolled steel sheet

for a press forming, which process comprises heating a cold-rolled steel sheet consisting essentially of

5 less than 0.08 wt. percent carbon  
0.05 to 0.4 wt. percent manganese  
0.015 to 0.10 wt. percent silicon  
0.003 to 0.015 wt. percent nitrogen

10 0.01 to 0.10 wt. percent acid-soluble aluminum the remainder being iron and unavoidable impurities, to a temperature in a range from 680° to 900°C and holding the same at this temperature for less than 10 minutes, subsequently cooling the steel sheet from the said temperature with a cooling rate of 5 to 54°C/sec. to the temperature of an overaging treatment, then subjecting the steel sheet to said overaging treatment, in which the steel sheet is held at a temperature of 300 to 500°C for less than 10 minutes and thereafter subjecting the steel sheet to a continuous annealing treatment, in which the steel sheet is quenched to room temperature.

20 2. The process of claim 1 wherein the overaging treatment is for 2 to 5 minutes.

25 3. A process for preparing a cold-rolled steel sheet for press forming, which includes vacuum degassing, whereby prior to cold rolling, the initial carbon content of a molten steel of 0.02 to 0.08 wt. percent is reduced to range of 0.001 to 0.009 wt. percent, which process comprises heating a cold-rolled steel sheet consisting essentially of

30 less than 0.08 wt. percent carbon  
0.05 to 0.4 wt. percent manganese  
0.015 to 0.10 wt. percent silicon  
0.003 to 0.015 wt. percent nitrogen

35 0.01 to 0.10 wt. percent acid-soluble aluminum the remainder being iron and unavoidable impurities, to a temperature in a range from 680° to 900°C and holding the same at this temperature for less than 10 minutes, subsequently cooling the steel sheet from the said temperature with a cooling rate of 5° to 54°C/sec. to the temperature of an overaging treatment, then subjecting the steel sheet to said overaging treatment, in which the steel sheet is held at a temperature of 300° to 500°C for less than 10 minutes and thereafter subjecting the steel sheet to a continuous annealing treatment, in which steel sheet is quenched to room temperature.

40 4. The product of the process of claim 1.

45 5. The product of the process of claim 3.

\* \* \* \* \*